

## UNITED STATES PATENT OFFICE

2,117,811

## TANNING

Gustav Mauthe and Hermann Noerr, Leverkusen-  
I. G. Werk, Germany, assignors to I. G. Far-  
benindustrie Aktiengesellschaft, Frankfort-on-  
the-Main, Germany

No Drawing. Application November 21, 1935,  
Serial No. 50,988. In Germany November 24,  
1934

6 Claims. (Cl. 149—4)

The present invention relates to an improvement in tanning and especially consists in an improved process for tanning with zirconium compounds.

5 It is known that zirconium salts display some tanning action and have, therefore, been proposed already for use as tanning agents in the leather industry. Now, of these salts, the one which can be obtained from zirconium minerals 10 most readily in a substantially pure and well defined state is the zirconiumoxychloride ( $ZrOCl_2 \cdot aq$ ) from which other zirconiumchlorides of different basicity can also easily be prepared. However, the affinity of zirconiumchlorides for 15 the animal skin fiber is rather small. Therefore, by the previously described tanning process making use of zirconiumchloride, it was not possible to prepare thoroughly tanned leathers; on the contrary, the products obtained according to the 20 said process are still of horny, parchment-like character and swell easily when treated with hot water.

It is the object of our invention to improve 25 tanning with zirconiumchlorides to such a degree that the resulting leathers will stand any competition in the market, thereby for the first time making practically possible the use of zirconiumchlorides in the leather industry, an achievement highly desirable for the above and 30 other reasons.

This object we attain by performing the tanning with zirconiumchlorides in the presence of sulfate ions, which are incorporated with the tanning liquor, for instance, by adding thereto 35 compounds yielding sulfate ions. Primarily sulfuric acid or watersoluble sulfates such, for instance, as sodium, potassium or aluminium sulfates may be mentioned as suitable compounds yielding sulfate ions, it being understood, however, that they are mentioned here only for examples' sake; so, if no value is set on a white color 40 of the leathers, chromium sulfates may be employed too. Furthermore, the said and other like sulfate compounds can be added alone or in combination with neutral salts.

The quantity of sulfate compounds and also 45 the manner of adding the same can vary somewhat, depending on the nature and kind of hides and the special tanning process employed. As 50 will be seen from the following examples they can easily be so chosen, however, by anyone skilled in the art, as to secure the optimum affinity of the tanning agent for the skin fiber. If, for instance, heavy hides are to be tanned, it is preferable to gradually add a sulfate or other sub-

stance yielding sulfate ions during the tannage, an amount of more than about 1% (calculated on the hide weight) being preferred. Tanning will then proceed softly and rapidly. On the other hand, with light skin material the whole amount of neutral salts necessary in order to prevent swelling can be added at the beginning in the form of water-soluble sulfates, for example, sodium sulfate.

In addition to the advantage of using the 10 easily obtainable zirconiumchlorides and, furthermore, the great adaptability to the kind of skin and the tanning process employed, it is another great advantage of our new process that, in comparison with the zirconium sulfate tannage, our 15 process can be performed at much higher basicity. For as is seen from the above formula, the easily water-soluble zirconiumchloride is 50% basic, a basicity not to be attained, for instance, with zirconium sulfate, as the corresponding basic sulfates are not soluble. But in spite of the high basicity the tanning according to our present 20 process is a mild one, especially if greater quantities of sulfate ions are employed, and yields full leathers of very fine grain. Besides, the quantity of the neutralizing agents to be added in the usual way at the end of the tannage in order to render the skin weakly acid, is considerably 25 smaller than the quantity necessary, for instance, in a zirconium sulfate tannage.

30 Our present process can be performed alone or in combination with other usual tanning processes.

The leathers obtainable according to our new 35 process are distinguished by their great fullness, light color and extraordinary fastness to light.

The following examples illustrate the invention 40 without limiting it thereto, the indications in percent being calculated upon the weight of the unhaired hides:—

## Example 1

Unlimed and bated unhaired goat hides are 45 thoroughly pickled in a pickle of hydrochloric acid and sodium chloride. The tannage is performed in 100% of water, 8% of sodium sulfate and 2.5% (calculated as zirconium dioxide) of  $ZrOCl_2 \cdot 8H_2O$ . The oxychloride is dissolved in a small amount of water and added in five portions during half a day. Tannage is continued 5 for some hours further until a test portion taken from the tanning liquor no longer yields any precipitate on the addition of an aqueous solution of sodium phosphate. The liquor is then gradually neutralized with an aqueous solution of about 1%

of sodiumbicarbonate until the reaction is only weakly acid to Congo red. The leathers are then beaten on the jack over night and rinsed the next day until the leather cut shows a pH value of 4.5; 5 they are then greased with a light-colored water-soluble fat and pole-dried. The finished leather shows a fine grain, a good fullness and a white color.

*Example 2*

10 A heavy, bated calf hide is drummed with about 2.8% of technical hydrochloric acid, 8% of sodiumchloride and 100% of water, until a homogeneous pickling is attained. Tannage is performed in a fresh liquor of 100% of water, 8% 15 of sodiumchloride and 7.8% of crystallized zirconiumoxychloride (corresponding to 3% of zirconiumdioxide). The oxychloride to be added is divided into four parts which are introduced into the liquor with intervals of half an hour. Tannage is continued for 3 hours further. 6% of anhydrous sodium sulfate is dissolved in water and divided into four parts and added with intervals of an hour. Drumming is continued for one to two hours. A streak cut from the leather and laid in water no longer shows any untanned swelling zone. The liquor is then neutralized with 0.6% aqueous solution of sodium bicarbonate. The leather is then beaten on the jack over night, rinsed in the drum with running water, greased, dried and worked up in the usual manner. The hydrochloric acid pickle may be replaced by a pickle of formic acid and sodiumchloride.

35 *Example 3*

Heavy calf hides which have been thoroughly pickled with hydrochloric acid are tanned with 7.8% of zirconiumoxychloride (3% of zirconiumdioxide), which, before adding to the tanning liquor, has been brought to a basicity of 25% with the aid of hydrochloric acid, in 100% of water in which 8% of anhydrous sodium sulfate is dissolved. The tanning agent is gradually added and tannage is continued until the thickest parts of the hides are thoroughly tanned. The liquor is neutralized with an aqueous solution of sodium bicarbonate until the reaction to Congo red is only weakly acid.

50 *Example 4*

A goat hide is cut in two halves and tanned in accordance with the manner described in Example 2 with the quantity of zirconiumoxychloride which corresponds to 2.5% of zirconiumdioxide. Instead of the addition of sodium sulfate as described in Example 2, (a) 6% of potassium sulfate or (b) 8% of aluminium sulfate is gradually added. In either case the tannage is continued until the zirconium reaction is negative, 55 when a thorough tanning is achieved. The liquor is then neutralized and the leathers are worked up in the usual manner. In both cases, very fine, soft and full leathers are obtained.

*Example 5*

Skivers are well pickled with formic acid and then tanned on the paddle for one to two days in a liquor of the following composition: 800% of water, 40% of sodiumchloride, 10% of zirconiumoxychloride, 1% of formic acid (technical 5 85%), 40% of anhydrous sodium sulfate.

After the leather is thoroughly tanned it is well rinsed, fatted, dried, moistened, dressed and 10 tacked.

*Example 6*

Cow hides are well pickled with hydrochloric acid and treated in the suspender with a liquor of the following composition: 200% of water, 5% 15 of zirconiumoxide in the form of zirconiumoxychloride, 20% of anhydrous sodium sulfate and 2% of technical hydrochloric acid (22%).

After two to three days the hides are thoroughly tanned. They are freed from the acid by 20 washing with water, oiled off, tacked and dried.

We claim:—

1. In the process of tanning with zirconium salts, the modification which comprises treating pickled hides of acid reaction with a solution 25 containing a water-soluble zirconium chloride and gradually adding thereto a water-soluble sulfate during tannage.

2. In the process of tanning with zirconium salts, the modification which comprises treating 30 pickled hides of acid reaction with a solution containing a water-soluble zirconium chloride and gradually adding thereto a water-soluble sulfate during tannage so that at the end more than about 1% of sulfate ions are present in the solution. 35

3. In the process of tanning with zirconium salts, the modification which comprises dissolving a water-soluble zirconium chloride and a water-soluble compound yielding sulfate ions in an 40 aqueous medium, and tanning pickled hides of acid reaction therein.

4. In the process of tanning with zirconium salts, the modification which comprises dissolving a water-soluble zirconium chloride and a water-soluble sulfate in an aqueous medium, and tanning 45 pickled hides of acid reaction therein.

5. In the process of tanning with zirconium salts, the modification which comprises dissolving a water-soluble zirconium chloride and a water-soluble sulfate selected from the group consisting of alkali metal and ammonium sulfates in an 50 aqueous medium, and tanning pickled hides of acid reaction therein.

6. In the process of tanning with zirconium salts, the modification which comprises dissolving zirconiumoxychloride ( $ZrOCl_2 \cdot aq$ ) and a water-soluble sulfate selected from the group consisting of alkali metal and ammonium sulfates in an 55 aqueous medium, and tanning pickled hides of acid reaction therein. 60

GUSTAV MAUTHE.  
HERMANN NOERR.